

Feb. 24, 1925.

1,527,250

L. EMANUELI

CABLE FOR CONVEYANCE OF ELECTRICAL ENERGY WITH GRADUATED INSULATION

Filed Nov. 22, 1921



Luigi Emanueli, <sup>Inventor</sup>  
By *Emil Barnelyckz,*  
<sup>Attorney</sup>

## UNITED STATES PATENT OFFICE.

LUIGI EMANUELI, OF MILAN, ITALY, ASSIGNOR TO SOCIETÀ ITALIANA PIRELLI, OF MILAN, ITALY.

## CABLE FOR CONVEYANCE OF ELECTRICAL ENERGY WITH GRADUATED INSULATION.

Application filed November 22, 1921. Serial No. 517,099.

*To all whom it may concern:*

Be it known that I, LUIGI EMANUELI, a subject of the King of Italy, residing at Milan, Italy, have invented certain new and 5 useful Improvements in Cables for Conveyance of Electrical Energy with Graduated Insulation, of which the following is a specification.

At present cables used for the conveyance 10 of electrical energy are almost always insulated by means of paper impregnated with suitable mixtures possessing high insulating power and great dielectric strength. A long series of investigations has demonstrated 15 the existence of a definite relation between the dielectric strength of impregnated paper and the mechanical permeability of paper to fluids.

The above mentioned permeability, the 20 co-efficient of which may be indicated by  $A$ , is determined by means of a special apparatus, in which air may be utilized as the working fluid. This apparatus may comprise an open-ended glass cylinder, of 25 known capacity, having its lower part immersed in a colored liquid. The air contained in the cylinder is exhausted from the top by means of an aspirator in such a manner that it must penetrate a small disk of 30 testing paper. The colored liquid then rises in the cylinder and fills the space  $V$  left by the air withdrawn. The time  $t$  necessary is calculated, and by means of a manometer the suction action  $P$  exerted on the paper 35 disk by the aspirator is measured. The co-efficient  $A$  which has been adopted to characterize the degree of permeability is determined by the formula

$$40 \quad A = \frac{PV\Omega t}{tsn},$$

in which  $\Omega$  and  $s$  respectively represent the surface and the thickness of the paper disk, while  $n$  is the coefficient of viscosity of the 45 fluid (air) employed in making the test. The dielectric strength of the paper can be determined by any of the well known methods.

The principal result of these experiments 50 is, that with the same mixture or oil for impregnating the paper the strength is found to be, up to a certain point, greatest in the papers least permeable to liquids. For example a type of paper which is very permeable ( $A=50,000$ ), is perforated after hav-

ing been impregnated with oil, at 15,000 volts per m.m; whilst, with a paper only very slightly permeable ( $A=370,000$ ), is similarly treated, a tension of 47,000 volts per m.m. may be attained before perforation. 60 However no further augmentation of dielectric strength is obtained with papers still less permeable.

In order therefore to obtain a high resistance against perforation in cables for conveying electrical energy, at very high tension it would be necessary to use only paper possessing a very low degree of mechanical permeability to liquids or at least not beyond a certain limit ( $A=400,000$ ). But this not 70 only prolongs the time for the impregnating operation very considerably but it also results in a considerable increase in the net cost, and furthermore it is necessary to conduct this operation with the greatest care, in 75 order that the paper shall not be exposed to a deterioration due to a long immersion in the mixture at a high temperature. Now since with high tension cables the distribution of the electric field is such that the risk 80 to which the insulation is exposed is greatest in the parts of the insulating cover which are in closest proximity to the conductor, the use of paper possessing a low degree of permeability may be confined to the layers 85 which are closest to the conductor, whilst for the outer layers a paper of higher permeability may be used. By these means it is possible to benefit by the result obtained during the course of the experiments mentioned above thus realizing an economical 90 technological advance.

The object of this invention is a new type of high tension cable insulated by means of impregnated paper, in which, from the conductor outwards, papers are employed of constantly increasing mechanical permeability to the oil or other liquid insulating material. Owing to this graduation, the insulation which is in immediate contact with 100 the conductor possesses a high dielectric strength, while this strength decreases towards the exterior layers; said exterior layers however, possessing great permeability, do not excessively prolong the duration of 105 the impregnation of the cable.

The single figure of the accompanying drawing is a sectional view of a cable constructed in accordance with the invention: 110 1 designating the conductor, 2 the inner

paper layers of high dielectric strength, 2<sup>2</sup> the outer paper layers of low dielectric strength, and 3 the protective sheath or coating.

5 Having now particularly described and ascertained the nature of my said invention and in which way the same is to be performed I declare that what I claim is:

1. An electric cable, comprising a conductor; layers of impregnated paper rolled upon the conductor, the mechanical permeability of said layers to the substance with

which they are impregnated increasing from the innermost layers outwards; and a protective sheath encasing said layers.

15

2. An electric cable provided with a succession of layers of paper impregnated with an insulating liquid and rolled one upon another, the mechanical permeability of said layers to the insulating liquid increasing 20 constantly, commencing with the innermost layers.

In testimony whereof I affix my signature.  
L. EMANUELI.